

Oct. 29, 1940.

W. E. JOMINY

2,219,780

ALLOY STEEL

Filed Jan. 6, 1938



Inventor  
Walter E. Jominy  
By  
Blackmar, Spencer & Flint  
Attorneys

## UNITED STATES PATENT OFFICE

2,219,780

## ALLOY STEEL

Walter E. Jominy, Detroit, Mich., assignor to General Motors Corporation, Detroit, Mich., a corporation of Delaware

Application January 6, 1938, Serial No. 183,573

3 Claims. (Cl. 75—123)

This invention relates to ferrous metal alloys and more particularly to alloy steels.

In many uses of articles formed of steel the property of depth hardness is a highly desirable characteristic. By depth hardness is meant the property of steel to become hardened in the heat treating operation to a distance below the surface. Since the rate of cooling of an article is slower below the surface than at the surface and becomes less as the center of the article is approached, it follows that a steel which hardens to the center of the article will harden with a slower rate of cooling than one which hardens only at the surface or slightly below. The depth hardening characteristics of steel then become really a matter of required speed of cooling to produce full hardening. One of the principal reasons for using alloy structural steels is to obtain deep hardening characteristics and if it were not for this property of alloy steels the plain carbon steels which are much lower in price could often be substituted for them. The deep hardening steels, since they can be hardened with a lower cooling speed, may be hardened in at least the moderate section sizes by quenching in oil. An article which can be hardened by quenching in oil will, in general, be less distorted and have lower internal stresses than one quenched in water or other more drastic quenching media.

In fact, for some automotive parts like ring gears, transmission gears and drive pinions, so much distortion occurs with water quenching that it is commercially impractical to harden by water quenching.

In order to obtain steels with proper hardening properties, certain alloy steels have been heretofore proposed. Due to the cost of the alloying ingredients used, the alloy steels are commonly quite expensive. I have found that with a steel of the composition of my invention, the cost is materially reduced as compared with the alloy steels of the prior art. Accordingly, it is one object of my invention to provide an alloy steel having good depth hardening properties that is much more economical to manufacture than previously known alloy steels of similar characteristics. Other objects of my invention are to provide an alloy steel adapted for a wide variety of uses that is cheaper and more economical than expensive alloy steels heretofore employed; to provide a steel having excellent properties of fatigue resistance; to provide an alloy steel especially adapted for use in parts to be case carburized and to provide a case carburized article of alloy steel in which

there is substantially no hypereuctectoid carbon in the case portion thereof.

Other objects and advantages of my invention will become more apparent from the following detailed description.

My invention comprises an alloy steel consisting of carbon, manganese, silicon, molybdenum and iron as essential alloying ingredients. In addition, small amounts of impurities such as phosphorus, sulphur, etc., may be present. Generally, the impurities will be present in amounts comparable with known steels and should not be present in such quantities as to impart objectionable characteristics or unduly retard the beneficial effects of the other alloying constituents. My improved alloy consists in the use of molybdenum in smaller amounts than heretofore considered commercially feasible in steels to be hardened so far as I am aware. The use of molybdenum in the range later outlined in combination with controlled amounts of silicon, manganese, carbon and iron results in a steel having improved properties in accordance with the invention.

In order to compare the depth hardening characteristics of the steel of my invention with various commercial steels, I have developed a test specimen and test procedure. Referring to the drawing there is shown a test specimen 10, one inch in diameter and three inches long. It has a cup-shaped portion 12 at one end and a screw-threaded opening 14 at the other. An adapter 16 connected to the screw-threaded end of the test bar secures the latter to a bracket 20. The bracket holds the test specimen in such a way that the cupped end is directly over a nozzle 22. The test specimen is hardened by heating to the desired temperature and then cooling by spraying water into the cupped end and directly cooling this face only as shown in the drawing. A receptacle 24 collects the water used in the cooling operation. After the specimen is cooled it is removed from the fixture, a strip of metal is removed by grinding to a depth of .015", and the hardness measured at various points along this ground surface from the water cooled end to the adapter end. From these readings the hardening characteristics of the steel are ascertained. For carburizing steels, the distance from the water cooled end, over which the hardness is 600 Vickers Brinell or above after carburizing and cooling on the fixture, is taken as a measure of the hardening characteristics of the steel. A number of the more common carburizing steels have been tested in this way to show their relative hardness characteristics and

some of these are included in Table 1. There are also included in Table 1 some of the steels of my invention and it will be seen that the hardenability characteristics of these steels compare favorably with those of the alloy steels listed.

TABLE 1

| 10 | S. A. E. steel         | Per-cent<br>C | Per-cent<br>Mn | Per-cent<br>Cr | Per-cent<br>Ni | Per-cent<br>Mo | Per-cent<br>Si | Per-cent<br>P | Per-cent<br>S | McQuaid-Ehn<br>grain size | Distance from<br>water cooled<br>end where<br>hardness is<br>600 Vickers<br>Brinell or<br>above |
|----|------------------------|---------------|----------------|----------------|----------------|----------------|----------------|---------------|---------------|---------------------------|-------------------------------------------------------------------------------------------------|
| 15 | 1020                   | .19           | .49            |                |                |                |                | .025          | .031          | 6-7                       | Inches                                                                                          |
|    | 1120                   | .20           | .55            |                |                |                |                | .101          | .189          | 3-4                       | $\frac{1}{16}$                                                                                  |
|    | 2315                   | .18           | .67            |                | 3.63           |                |                | .025          | .019          | 3-4                       | $\frac{3}{16}$                                                                                  |
|    | 3115                   | .14           | .50            | .68            | 1.08           |                |                | .025          | .029          | 5                         | $\frac{1}{2}$                                                                                   |
|    | 4315                   | .19           | .69            | .54            | 1.95           | .30            | .22            | .025          | .012          | 6-8                       | $\frac{3}{16}$                                                                                  |
|    | 4615                   | .19           | .52            |                | 1.88           | .27            |                | .025          | .017          | 6-8                       | $\frac{1}{16}$                                                                                  |
|    | 5115                   | .14           | .70            | .94            |                |                |                | .025          | .025          | 6                         | $\frac{1}{16}$                                                                                  |
| 20 | Steels of my invention |               |                |                |                |                |                |               |               |                           |                                                                                                 |
|    | 61                     |               | .23            | .90            |                |                |                | .10           | 1.07          |                           |                                                                                                 |
|    | 76                     |               | .18            | .94            |                |                |                | .05           | 1.03          |                           |                                                                                                 |
|    | 60                     |               | .26            | 1.20           |                |                |                | .10           | 1.10          |                           |                                                                                                 |
|    | 66                     |               | .25            | 1.14           |                |                |                | .18           | 1.27          |                           |                                                                                                 |
| 25 | 53                     |               | .22            | 1.09           |                |                |                | .18           | 1.08          |                           |                                                                                                 |
|    | 89                     |               | .35            | 1.23           |                |                |                | .05           | 1.06          |                           |                                                                                                 |
|    | C-53                   |               | .22            | 1.09           |                |                |                | .18           | 1.08          |                           |                                                                                                 |
|    | C-60                   |               | .27            | 1.20           |                |                |                | .10           | 1.10          |                           |                                                                                                 |
|    | C-77                   |               | .20            | .98            |                |                |                | .05           | .53           |                           |                                                                                                 |
|    | C-89                   |               | .21            | 1.00           |                |                |                | .05           | .96           |                           |                                                                                                 |

30 In the steel of my invention the three alloying constituents, manganese, silicon and molybdenum within the ranges disclosed, are essential to produce good depth hardness. I have made steels in which only two of the three are present 35 and when this is done substantially lower depth hardness is obtained. This may be observed from the following steels which were all tested for hardenability by carburizing eight hours at 1700° F. and cooling on the quenching fixture as 40 already explained.

| 45 | Steel | Per-cent<br>C | Per-cent<br>Mn | Per-cent<br>Si | Per-cent<br>Mo | Grain<br>size | Distance from<br>water cooled<br>end where<br>hardness is<br>600 Vickers<br>Brinell or<br>above | Inches         |
|----|-------|---------------|----------------|----------------|----------------|---------------|-------------------------------------------------------------------------------------------------|----------------|
| 50 | C-78  | .23           | .90            | 1.13           |                | 5-6           |                                                                                                 | $\frac{3}{16}$ |
|    | C-10  | .07           | .98            | .69            |                | 5-6           |                                                                                                 | $\frac{3}{16}$ |
|    | C-81  | .15           | .34            | .97            | .10            | 4-5           |                                                                                                 | $\frac{3}{16}$ |
|    | C-82  | .11           | .24            | .93            | .15            | 4-5           |                                                                                                 | $\frac{3}{16}$ |
|    | C-84  | .09           | .86            | Trace          | .10            | 5-6           |                                                                                                 | $\frac{3}{16}$ |
|    | C-86  | .07           | .99            | Trace          | .10            | 4-6           |                                                                                                 | $\frac{1}{16}$ |

55 It will be noticed that steels C-78 and C-10 in which the molybdenum was omitted have a low hardenability rating for alloy steels as compared with steels in accordance with my invention. This is also true of steels C-81 and C-82 in which 60 the manganese is kept low and is likewise true when the silicon is omitted as shown in steels C-84 and C-86. When, however, the manganese and silicon are within the desired range and as little as .05% molybdenum is added, a very definite increase in the hardenability characteristic of the steel is obtained, as indicated in the steels of my invention in Table 1. Further increase in molybdenum content gives additional increase in hardness penetration. Increase in 70 the manganese content with the same molybdenum likewise gives an increase in hardenability characteristic.

I have found that an alloy in accordance with my invention consisting of molybdenum .05-.15%, carbon .05-1.20%, manganese 0.90-1.60%, silicon

0.60-1.50%, balance iron plus minor amounts of impurities has good properties of depth hardening and good properties as regards fatigue resistance and is one that is economical in cost as compared with higher priced alloy steels. For 5 most purposes a narrower range of the several

|    |  |  |  |  |  |  |  |  |  |  |    |
|----|--|--|--|--|--|--|--|--|--|--|----|
| 10 |  |  |  |  |  |  |  |  |  |  | 10 |
| 15 |  |  |  |  |  |  |  |  |  |  | 15 |
| 20 |  |  |  |  |  |  |  |  |  |  | 20 |
| 25 |  |  |  |  |  |  |  |  |  |  | 25 |
| 30 |  |  |  |  |  |  |  |  |  |  | 30 |
| 35 |  |  |  |  |  |  |  |  |  |  | 35 |
| 40 |  |  |  |  |  |  |  |  |  |  | 40 |
| 45 |  |  |  |  |  |  |  |  |  |  | 45 |
| 50 |  |  |  |  |  |  |  |  |  |  | 50 |
| 55 |  |  |  |  |  |  |  |  |  |  | 55 |
| 60 |  |  |  |  |  |  |  |  |  |  | 60 |
| 65 |  |  |  |  |  |  |  |  |  |  | 65 |
| 70 |  |  |  |  |  |  |  |  |  |  | 70 |

|                                         |          |
|-----------------------------------------|----------|
| constituents is preferred, for example: | Per cent |
| Molybdenum                              | .05-.12  |
| Carbon                                  | .05-1.20 |
| Manganese                               | .95-1.30 |
| Silicon                                 | .90-1.25 |
| Iron plus minor amounts of impurities   | Balance  |

My new alloy is especially adapted for parts requiring case carburizing, for example, ring gears and the like. For this purpose the carbon content of the articles to be carburized will be preferably within the range .05-.30%. The combination of the several alloying elements in the amounts specified is such that an article formed from the alloy after carburizing has substantially no hypereutectoid carbon in the case. This permits quenching the article directly from the carburizing box, at say a temperature of 1700° F., for example, and obtaining a very hard martensitic surface of approximately eutectoid carbon concentration, whereas most alloy steels when similarly treated provide a softer austenitic surface of hypereutectoid carbon.

A steel made in accordance with my invention has a wide variety of uses in the construction of parts for automobiles where alloy steels are required due to severe conditions of operation. The steel of my invention is a steel of great strength and is resistant to fatigue. The manufacture thereof entails no special difficulties.

I claim:

|                                                                                                                                                    |          |
|----------------------------------------------------------------------------------------------------------------------------------------------------|----------|
| 1. A case carburized article having a core composed of the following elements as essential ingredients in substantially the following proportions: | Per cent |
| Carbon                                                                                                                                             | .05-.30  |
| Manganese                                                                                                                                          | .90-1.60 |
| Silicon                                                                                                                                            | .60-1.50 |
| Molybdenum                                                                                                                                         | .05-.15  |
| Iron                                                                                                                                               | Balance  |

said article having a case of approximately eutectoid carbon content.

2. A case carburized article having a core composed of the following elements as essential in-

gredients in substantially the following proportions:

|             | Per cent |
|-------------|----------|
| Carbon      | .05-.30  |
| 5 Manganese | .95-1.30 |
| Silicon     | .90-1.25 |
| Molybdenum  | .05-.12  |
| Iron        | Balance  |

5 10 said article having a case of approximately eutectoid carbon content.

10 3. A case carburized alloy steel article having a case of approximately eutectoid carbon concen-

tration obtained by treatment in a carburizing medium at a carburizing temperature and having a core containing .05-.30% carbon, the remaining composition of the case carburized article being .90-1.60% manganese, .60-1.50% silicon, .05-15% molybdenum and the balance iron plus minor amounts of impurities, said article when quenched direct from the carburizing medium at substantially the carburizing temperature having a hard, martensitic surface of approximately eutectoid carbon concentration.

WALTER E. JOMINY.